

## UNITED STATES PATENT OFFICE

ROBERT SCHLESS, OF EMPORIUM, PENNSYLVANIA

## EXPLOSIVE

No Drawing.

Application filed July 10, 1928. Serial No. 291,694.

This invention relates to explosives and more particularly explosives of the nitroglycerine type. In the ammonium nitrate class of permissible explosives of the above type, which are used mainly in gaseous and dusty coal mines, only a comparatively low percentage of nitroglycerine or its modifications can be used, and this low percentage of nitroglycerine or its modifications, makes the initiation and propagation sensitiveness of this type of explosive comparatively low, especially after storage. For example, the upper limit of nitroglycerine in such explosives is generally 12% and usually is 10%.

Further, while for various reasons, a low density explosive is desired in some coal mining operations, the general method of lowering density namely by increase in the amount of carbonaceous material, cannot be utilized with this type of explosive for the reason that a limit is reached such as from 10 to 12% of carbonaceous material beyond which a further increase interferes with the sensitiveness of the explosives. This may be defined in another way. Density as applied to mining explosives, is ordinarily expressed in terms of the number of 1 $\frac{1}{4}$  x 8" cartridges in fifty lbs. of the finished explosive and is dependent of course on the choice of ingredients, especially of the carbonaceous material, and on the manner in which the explosives are loaded or "packed" in the paper cartridges ordinarily used. With explosives normally in use for mining, regulating the choice and quantity of ingredients enables a maximum cartridge count of between 175 and 180 to be attained. However higher cartridge count is often desired and if this is attempted by the ordinary methods, the results are insensitive explosives which are a menace to safety and efficiency of blasting.

The use of sodium nitrate in explosive compositions has been somewhat limited due to its well known sluggish character inherent in its property of releasing its oxygen slowly. It would be of advantage to overcome this sluggishness as this would increase the initiation and propagation sensitiveness and

bring about more efficient and safer blasting especially in those cases where, due to peculiar conditions, as in coal mining, explosives of low nitroglycerine content were heretofore considered safe, other varieties being dangerous in such instances. Recent suggestions in the prior art to utilize sodium nitrate have been tied up with a simultaneous incorporation of ammonium nitrate as the principal impregnating agent as where carbonaceous material has been impregnated with ammonium nitrate prior to its admixture with sodium nitrate, or where adhesive blends of ammonium nitrate and sodium nitrate are first prepared. But it will be noted that these prior art suggestions are directed not to nitroglycerine type explosives, since in the first example referred to above no nitroglycerine was used, while in the case of the adhesive blends composition, a relatively low percentage of nitroglycerine—not over 5%—was used, which is customary with lower type of explosives in which this low percentage of nitroglycerine is used as sensitizing ingredient but not as the principal explosive ingredient.

Among the objects and advantages of the present invention, is the production of explosives of the nitroglycerine type of relatively low density or high cartridge count, which are sensitive, safe and efficient.

And more particularly an object of the present invention is the production of explosives of the character set forth above wherein a low density is obtainable without unfavorably affecting the sensitiveness of the explosives produced in accordance with this invention.

Other and further objects and advantages will appear from the more detailed description set forth below, it being understood however that this more detailed description is given by way of illustration and not by way of limitation, since various changes may be made therein by those skilled in the art without departing from the scope and spirit of this invention as herein set forth.

It has now been found that if the sodium nitrate is incorporated into the cells of the carbonaceous material and an explosive be

made including in its composition, a sufficient amount of nitroglycerine, or its modifications, to act as the principal detonating and sensitizing agent, satisfactory explosives 5 of the nitroglycerine type are obtainable, and the prior art difficulties heretofore encountered are eliminated.

To obtain the desired incorporation of the carbonaceous material with sodium nitrate, 10 the carbonaceous material may be mixed with water and then sodium nitrate added causing it to be dissolved in the water, the solution to be absorbed by the carbonaceous material, and the surplus water subsequently evaporated. Or the sodium nitrate may first 15 be dissolved in the water, the carbonaceous material then mixed with the solution in order to absorb said solution, and then the excess water evaporated therefrom. Or if desired, a solution of sodium nitrate may be 20 sprayed upon the desired carbonaceous material in a closed vessel in the presence of high pressure steam (say about 100 pound pressure), and the pressure then released so that the resultant expansion bursts the cells 25 of the carbonaceous material and the sodium nitrate is deposited within the material. Of course any other desirable method of impregnating the carbonaceous material with 30 the sodium nitrate may be utilized. The proportion of sodium nitrate to the material to be treated is variable depending on the density desired in the product.

The following example will serve as an 35 illustration of a method of making an explosive in accordance with the present invention. The carbonaceous material incorporated with sodium nitrate in a manner such as that set forth above and containing 30% of sodium nitrate to 70% of the carbonaceous material, the carbonaceous material in this example desirably being of the lowest available density is utilized in a composition containing:

|                       |     |
|-----------------------|-----|
| Nitroglycerine        | 14% |
| Carbonaceous material | 14% |
| Sodium nitrate        | 25% |
| Ammonium nitrate      | 46% |
| Calcium carbonate     | 1%  |

This admixture of materials using the lowest available density carbonaceous material,

yields an explosive of satisfactory sensitivity and having a cartridge count of about 205.

While the proportions given above are specific for the particular type of explosive 70 therein produced, the proportions may be varied considerably without affecting the principles of this invention.

Any desired carbonaceous material may be utilized, but for the production of explosives 75 of the lowest density, carbonaceous material of low density should be employed. Balsa wood may be desirably used in this connection, but the invention is not limited to a certain kind of carbonaceous material as the 80 treatment hereinabove set forth can be applied to a great variety of such materials having various densities and other characteristics.

As set forth above, nitroglycerine or its 85 modifications may be used in making the explosives referred to, and these modifications include nitrated solutions of sugar in glycerine, nitrated mixtures of glycerine and glycol, or glycerine and polyglycerine, or 90 glycerine and chlorhydrin, etc.

In the preferred explosives made in accordance with this invention, the amounts of nitroglycerine or its modification should not 95 fall below 8%.

Having thus set forth my invention, I claim:

1. In a process of making explosives, the steps of mixing a sodium nitrate solution with carbonaceous material under pressure, 100 and then releasing the pressure whereby the sodium nitrate is deposited within the cells of the carbonaceous material.

2. In a process of making explosives, wherein sodium nitrate solution and carbonaceous material are maintained under pressure, the step of releasing the pressure so that the sodium nitrate is deposited within the cells of the carbonaceous material.

3. In a process of making explosives, the steps of mixing a solution of a salt used in explosive compositions with carbonaceous material under pressure, and then releasing the pressure whereby the salt is deposited within the cells of the carbonaceous material.

ROBERT SCHLESS.